# EUROPEAN PATENT SPECIFICATION

(11) **EP 0 733 131 B1**
(45) Date of publication and mention of the grant of the patent: **06.08.1997**
(21) Application number: 95904768.9
(22) Date of filing: 30.11.1994
(51) Int. Cl.: D01F 6/92

(54) **MONOFILAMENT FOR PAPERMAKER'S FABRIC**
MONOFILAMENT FÜR PAPIERMASCHINENGEWEBE
MONOFILAMENT POUR TOILE DE FABRICATION DU PAPIER

(30) Priority: 08.12.1993 US 163885
(43) Date of publication of application: 25.09.1996
(73) Proprietor: Asten, Inc., Charleston South Carolina 29423-8001 (US)
(72) Inventor: REITHER, John, R., Summerville, SC 29485 (US)
(74) Representative: Boydell, John Christopher
(86) International application number: US9413725
(87) International publication number: WO9516064

(56) References cited:
- DE-B- 1 222 205
- DE-C- 4 307 392
- DATABASE WPI Section Ch, Week 9442, Derwent Publications Ltd., London, GB; Class A, AN 94-339179 ANONYMOUS 'Prodn of improved monofilament - by blending polycarbonate with 1,4-cyclo:hexane:di:methane contg polyester(s)'
- DATABASE WPI Section Ch, Week 8138, Derwent Publications Ltd., London, GB; Class A, AN 81-68844D

## Description

### FIELD OF THE INVENTION

The present invention relates generally to monofilament yarns for industrial fabric, and especially to yarns for use in papermaking fabrics.

### BACKGROUND OF THE INVENTION

Generally, in the process for making paper, incremental amounts of liquid are removed from a slurry of pulp in a succession of steps. In a first forming step, the slurry is deposited on a porous fabric which drains much of the liquid by gravity and suction and leaves a wet web of solids on the fabric surface. In a later pressing step, the wet web is typically compressed between fabrics to remove additional liquid. In a still later, drying step more liquid is removed by evaporation, usually by supporting the web by dryer fabrics so that the web is contacted with large diameter, smooth, heated rolls.

Papermaking places considerable demands on the fabrics used in each process step. The fabrics should be structurally strong, flexible, abrasion resistant and able to resist the harsh chemicals and high temperatures to which they can be exposed for extended times.

One major improvement in papermaking fabric technology has been the use of synthetic polymer monofilaments. Use of polymer, however, presents additional design constraints. For example, the polymer must be commercially processable to form monofilament of uniform quality. Furthermore, the polymer must make a monofilament that is sufficiently strong and impact resistant for automated fabric manufacturing techniques, as well as, for running on papermaking machinery at high speed.

Monofilaments have been made from such polymers as polyethylene terephthalate (PET) and polyphenylene sulfide (PPS). Each has physical properties which affect its suitability for papermaking fabric. PET has good dimensional stability, reasonable resistance to abrasion, is moderately priced but has marginal hydrolytic stability. PPS monofilament has excellent hydrolytic stability but is very expensive, highly crystalline, relatively brittle, and exhibits low knot and loop strengths.

It is desired to provide a low cost, strong, polymeric monofilament for industrial fabrics, which meets the demands of papermaking, including high knot strength and good hydrolytic stability. It is also desired to provide a monofilament which is suitable for use in the automated manufacturing process for such fabrics.

### SUMMARY OF THE INVENTION

The present invention provides high knot strength, hydrolysis resistant monofilament for use in papermaker's fabric. More specifically, there is provided a monofilament of a polymer blend consisting essentially of:
(a) 1-10 weight percent of a polyester selected from the group consisting of (1) polycarbonate and (2) glycol-modified copolyester comprising recurring units of copolymerized cyclohexane-1,4-dimethanol and copolymerized terephthalic acid, and recurring units of a copolymerized glycol other than cyclohexane-1,4-dimethanol and copolymerized terephthalic acid; and
(b) a complementary amount to total 100 weight percent of acid-modified copolyester comprising recurring units of copolymerized cyclohexane-1,4-dimethanol and copolymerized terephthalic acid, and recurring units of copolymerized cyclohexane-1,4-dimethanol and copolymerized dicarboxylic acid other than terephthalic acid.

There is also provided a papermaker's fabric of yarns including the above-described monofilament.

There is further provided a process for making a papermaker's fabric using the above-described monofilament.

### BRIEF DESCRIPTION OF THE DRAWINGS

The Figure is a graph of the percent retained knot strength (A) and the percent coefficient of variation of retained knot strength (B), plotted against the weight percent polycarbonate in a monofilament of one embodiment of the present invention.

### DETAILED DESCRIPTION OF THE PREFERRED EMBODIMENTS

The polymer blend suitable for the monofilament of this invention consists essentially of two polymers. The term "consists essentially of" as used herein means that the blend can include other components; provided that such components do not significantly detract from the function or operability of the invention. The term "monofilament" as used herein means a single fiber structure and is used interchangeably with the term "yarn".

One polymer of the blend is an acid-modified copolyester, occasionally hereinafter referred to as PCTA. It is a semicrystalline thermoplastic copolymer substantially of two recurring units. One such recurring unit is of copolymerized cyclohexane-1,4-dimethanol (CHDM) and copolymerized terephthalic acid. The other recurring unit is of copolymerized CHDM and a copolymerized dicarboxylic acid other than terephthalic acid. Thus, recurring units are according to the following formulae (I) and (II), respectively: wherein
- CHDM': is a radical obtained by dehydroxylation of CHDM;
- AR1: is a radical of decarboxylated terephthalic acid; and
- AR2: is a radical obtained by decarboxylation of a dicarboxylic acid other than terephthalic acid.

PCTA can be prepared either by direct polyesterification of CHDM with an appropriate mixture of dicarboxylic acids, or by transesterification of dialkyl esters of dicarboxylic acids with an effective amount of CHDM followed by polycondensation. Preferred other dicarboxylic acids include, for example, isophthalic acid and phthalic acid. Thus, PCTA is seen to be a copolyester of poly(cyclohexane-1,4-dimethylene terephthalate) wherein a portion of the terephthaloyl radical is replaced by isophthaloyl or phthaloyl radicals.

The amount of recurring unit (I) is from about 10-99 mole percent, preferably 50-99 mole percent, and more preferably, about 90-97 mole percent of the total of recurring units (I) and (II).

The second polymer of the blend is polycarbonate or a glycol-modified copolyester, occasionally hereinafter referred to as PCTG. PCTG is a semicrystalline thermoplastic copolymer substantially of two recurring units. One such recurring unit is of copolymerized CHDM and copolymerized terephthalic acid in accordance with formula (I). The other recurring unit is of a copolymerized glycol other than CHDM and copolymerized terephthalic acid, according to the following formula (III) : wherein
- R: is an organic radical containing 2-20 carbon atoms obtained by dehydroxylation of a linear, branched or cyclic aliphatic bifunctional glycol or ether glycol.

Illustrative examples of bifunctional glycols suitable for use in the glycol-modified copolyester component are ethylene glycol; 1,4-butanediol; 1,5-pentanediol and 1,10-decanediol. Illustrative examples of ether glycols are diethylene glycol and triethylene glycol. Ethylene glycol is preferred.

PCTA, PCTG and the method for making them are more fully described in U.S. Patent 2,901,466.

Polycarbonate suitable for use in the present invention includes carbonate polymers of dihydric phenols as well as carbonate copolymers of glycols, such as, for example, ethylene glycol or propylene glycol; dibasic acids, such as, for example, isophthalic or terephthalic acid; and hydroxyl or acid-terminated polyesters, such as, for example, the hydroxyl or acid-terminated polyester of neopentyl glycol and adipic acid. Such polycarbonate resins may be prepared by reacting a dihydric phenol with a carbonate precursor such as phosgene, a haloformate or a carbonate ester. Generally the resulting carbonate polymers may be typified as having recurring units of the following formula (IV): wherein A is a divalent aromatic radical of the dihydric phenol, preferably 4,4'-isopropylidenebisbenzenol, (bisphenol A), employed in the polymer producing reaction. The dihydric phenols which may be employed to provide such aromatic carbonate polymers are mononuclear or polynuclear aromatic compounds, containing as functional groups, two hydroxyl radicals, each of which is attached directly to a carbon atom of an aromatic nucleus. Typical dihydric phenols are 2,2-bis-(4-hydroxyphenyl)-propane; 1,3-benzenediol; 1,4-benzenediol; 2,2-bis-(4-hydroxyphenyl)-pentane; 2,4'-dihydroxydiphenyl methane; bis-(2-hydroxyphenyl)-methane; bis-(4-hydroxyphenyl)-methane; bis-(4-hydroxy-5-nitrophenyl)-methane; 1,1-bis-(4-hydroxyphenyl)-ethane; 3,3-bis-(4-hydroxyphenyl)-pentane; 2,6-dihydroxynapthalene; bis-(4-hydroxyphenyl)-sulfone; 2,2'-dihydroxydiphenyl sulfone; 4,4'-dihydroxydiphenyl ether; and 4,4'-dihydroxy-2,5-diethoxydiphenyl ether. It is, of course possible to employ two or more different dihydric phenols or, as stated above, a dihydric phenol in combination with a glycol, a hydroxy or acid-terminated polyester, or a dibasic acid in the event a carbonate copolymer rather than a homopolymer is desired.

The monofilament of the present invention can be prepared using conventional monofilament production equipment. The components of the polymer blend are typically supplied as particles in granular or pellet form. They should have a low moisture content to avoid degradation during subsequent melt processing. The particles can be melt blended continuously, in equipment such as single screw and twin-screw extruders, or batchwise in Banbury™ or Brabender™ mixers.

It has been found advantageous to make the monofilament in a two-step process. In such a process, a melt-blended masterbatch containing a conveniently high concentration of the minor component in PCTA is prepared. The masterbatch is pelletized and the pellets are later melt blended with additional PCTA to provide monofilament of desired composition. This two-step process provides good uniformity of composition, particularly when the product contains small amounts of the minor component, *i.e.*, 5 weight percent or less.

Monofilament of this invention should be made by when the melt blending at lower shear conditions than is conventional in polymer melt blending operations. Reduced shear averts polymer degradation during melt processing. Low shear can be achieved by known methods such as slowing the processor screw speed or using a low compression ratio screw. Normally, this is accompanied by a compensating reduction in production rate to achieve a uniform blend. The minor component should be uniformly dispersed throughout the composition.

Typically the melt is filtered through a screen pack, extruded through a multihole die, quenched to produce strands, drawn and heat-set to form monofilament. The drawing and heat-setting can include multiple cycles at different draw ratios and temperatures and can include one or more relaxation steps. Monofilament for papermaker's fabric typically has a diameter in the range of about 0.1 to 1.5 mm.

The monofilament of the present invention can be made into industrial fabric by conventional methods. It can be woven on looms in the traditional warp and fill fabric structure or formed into spiral structure in which parallel spiral monofilaments are intermeshed with pintle yarns. The fabric of this invention can be formed exclusively from the novel monofilament or from the novel monofilament in combination with other materials. A preferred use for the fabric of this invention is in papermaking machines.

Monofilament from PCTA blends of this invention provides high retained knot strength in combination with good hydrolysis resistance at reasonable cost. PCTA, absent added polymer blend components as herein provided, has hydrolysis resistance superior to PET but only moderate knot strength because it is brittle. Incorporation of small amounts of polycarbonate or glycol-modified copolyester into PCTA dramatically improves retained knot strength, while maintaining hydrolysis resistance, and without substantially adversely affecting other physical properties. It is now also revealed that the coefficient of variation of retained knot strength of the blended composition yarn is, unexpectedly, significantly less than that of wholly PCTA yarn. Consequently, the yarn of this invention is not only more ductile than PCTA yarn, but it can resist breaking during fabric forming and papermaking operations more consistently, and with better predictability, than PCTA yarn.

The present invention can be more fully understood by reference to the following representative examples of certain preferred embodiments thereof, where all parts, proportions and percentages are by weight unless otherwise indicated.

### EXAMPLES

In the following examples, tensile strength and related properties were measured on a tensile testing machine operated with 25.4 cm/minute (10 inch/minute) jaw separation rate and 25.4 cm (10 inch) initial jaw separation. Modulus was measured as the slope of the stress/strain curve at 1 percent strain. Free shrink was measured as percent dimensional change after unrestrained exposure to 204°C (400°F) for 15 minutes. Hydrolysis resistance was measured as percent of initial tensile strength at break retained by the sample after 5 hours of exposure to steam at 163°C (325°F).

### Examples 1 and 2 and Comparative Example C1

LEXAN™ 141 polycarbonate from General Electric, hereinafter "PC", and KODAR™ "Thermx 13319" PCTA from Eastman Chemicals, hereinafter "Polymer A", pellets were mixed to obtain mixtures of 5 % and 10 % PC in Polymer A. In separate runs, each mixture was fed to a 1.5 inch single screw extruder equipped with a general purpose screw operating at 24.7 rpm and 289°C (552°F) to obtain a melt blend. The melt blends were filtered through a 250 mesh (70 µm) screen pack and extruded through a multihole die. The extrudate was quenched under water and drawn to a ratio of 3.82:1, to produce a yarn of 0.4 mm diameter. Some volatiles generated during extrusion, perhaps from insufficient drying of the materials, caused the yarn to break frequently during quenching and drawing. Extrusion was steady, however. Polymer A, without PC, was similarly processed to produce comparison yarn C1.

Samples of each yarn were tested for retained knot strength by the following method. Tensile strength at break was determined. Knotted breaking strength was measured as the tensile strength at break after placing an overhand knot in fresh a test sample. Retained knot strength was calculated as the knotted breaking strength expressed as a percentage of the tensile strength at break. Retained knot strengths of Example 1 samples were about 50 %, which compared favorably to only 10-15 % observed for yarn C1.

### Examples 2-5 and Comparative Example C2

PC and Polymer A were dried at 121°C (250°F) for 6 hours to less than 0.02 % moisture and tumbled to obtain a 30 % PC mixture. The mixture was continuously melt blended at 102 kg (225 pounds) per hour in a twin-screw extruder equipped with a vacuum vent port and operated at 381 mm (15 inches) Hg, to obtain 400 pounds of masterbatch. The screw speed was 312 rpm and the extruder zones 1-6, die and melt temperatures were 266°C, 271°C, 260°C, 254°C, 254°C, 254°C, 268°C and 257°C (510, 520, 500, 490, 490, 490, 515 and 495°F), respectively. The melt blend was extruded as strand, quenched and cut to pellets. The masterbatch pellets were crystallized in pans at 177°C (350°F) for 2.5 hours.

Masterbatch pellets were dried at 121°C (250°F) for 5 hours then fed to an extruder with polymer A to obtain 0, 3.2, 4.5, 7.3 and 10.0 % PC compositions, Examples C2 and 2-5, respectively. The compositions were extruded at 24.8 rpm screw speed in a 8.9 cm (3.5 inch) single screw extruder operated at exit melt temperature in the range of 293-299°C (560-570°F). The compositions were extruded through a multihole spinneret with 2.0 mm diameter and 4.0 mm capillary length holes. The extrudate was quenched in water and dried. It was then drawn and relaxed in a succession of stages to a ratio of 3.45:1 to provide 0.5 mm diameter monofilaments. Extrusion and spinning of the low PC concentration yarns went smoothly. At 10 % PC, polymer began to build up on the die and to drip into the yarn. Physical properties of the yarns are shown in Table 1.

**Table 1**

| **Example** | **C2** | **2** | **3** | **4** | **5** |
|---|---|---|---|---|---|
| PC, % | 0 | 3.2 | 4.5 | 7.3 | 10 |
| denier | 2251 | 2200 | 2212 | 2222 | 2249 |
| elongation at 1.75 grams per denier, % | 11.1 | 12.6 | 13.9 | 18.1 | 22.6 |
| breaking energy, kg-mm | 243.9 | 254.4 | 275.5 | 307 | 321.6 |
| tenacity, grams/denier | 2.89 | 2.81 | 2.75 | 2.52 | 2.33 |
| breaking elongation, % | 23.7 | 25.9 | 28.3 | 33.4 | 37.2 |
| modulus, grams/denier | 37.9 | 37.8 | 36.9 | 34.4 | 32.4 |
| elongation at 1 pound, % | 0.55 | 0.54 | 0.54 | 0.58 | 0.61 |
| free shrink, % | 4.7 | 6.1 | 6.1 | 5.8 | 5.9 |
| retained knot strength, % | 40.4 | 69.7 | 65.5 | 74.2 | 73.3 |
| retained knot strength variability, %COV* | 37.2 | 14.2 | 14.4 | 9.5 | 3.1 |

| | | | | | |
|---|---|---|---|---|---|
| * coefficient of variation | | | | | |

Above 4.5 % PC, tenacity and modulus decrease. However, as the concentration of PC increases, toughness which is indicated by breaking energy and retained knot strength, increases. Retained knot strength of Examples 2-5 were substantially higher than those of C2. Above 4.5 % PC, retained knot strength remains levels at about 70 %. The coefficient of variation of retained knot strength, calculated by dividing the standard deviation of 10 replicates by the average, drops as PC concentration increases. The smaller coefficients of variation show that retained knot strength of the yarn from blends was less variable than PCTA yarn and that consistency of retained knot strength improves with increasing PC content. Knot strength improvement data from Table 1 is shown graphically in the Figure. The ordinate is percent property value and the abscissa is percent PC in the yarn. Line A represents retained knot strength and Line B represents coefficient of variation.

### Examples 6 and 7

A masterbatch of 30 % KODAR™ 5445 PCTG from Eastman Chemicals, hereinafter "Polymer G" and 70% Polymer A was prepared as in Examples 2-5. Extruder zones 1-6, die and melt temperatures were 260, 266, 254, 249, 249, 249, 266 and 254°C (500, 510, 490, 480, 480, 480, 510 and 490°F), respectively. Screw speed was 325 rpm and production rate was 100 kg (220 pounds) per hour.

The masterbatch was processed as in Examples 2-5 except that extruder exit melt temperature was in the range of 285-291°C (545-555°F) and the compositions were 3 and 6% PCTG, Examples 6 and 7, respectively. Analytical results are presented in Table 2.

**Table 2**

| **Example** | **6** | **7** | **8** | **C3** |
|---|---|---|---|---|
| PCTG, % | 3 | 6 | 3 | 0 |
| draw ratio | 3.8:1 | 3.8:1 | 4.2:1 | 4.2:1 |
| denier | 2224 | 2224 | 2220 | 2214 |
| elongation at 1.75 grams/denier, % | 11.6 | 11.9 | 8.4 | 8.1 |
| breaking energy, kg-mm | 261.7 | 265.9 | 219 | 206.8 |
| tenacity, grams/denier | 2.88 | 2.84 | 3.23 | 3.24 |
| breaking elongation, % | 25.4 | 25.9 | 19.9 | 19.0 |
| modulus, grams/denier | 38.1 | 39.3 | 43.8 | 44.0 |
| elongation at 1 pound, % | 0.53 | 0.52 | 0.48 | 0.47 |
| free shrink, % | 4.1 | 3.7 | 6.1 | 6.5 |
| retained knot strength, % | 64.6 | 59.8 | 58.9 | 27.7 |
| knot strength variability, % COV* | 18.0 | 17.5 | 6.8 | 51.5 |

| | | | | |
|---|---|---|---|---|
| * coefficient of variation | | | | |

Relative to Comparative Example C2 (Table 1) retained knot strength increased from 40.4 % to about 60 %, representing a 50 % improvement. Furthermore, the coefficient of variation of retained knot strength dropped dramatically, indicating that knot strength of the yarn from blends was much more consistent than yarn of PCTA alone. Other yarn properties were not significantly affected by incorporation of PCTG.

### Example 8 and Comparative Example C3

The procedures of Examples 6 and C2 were repeated except that the first stage draw ratio was increased from 3.8:1 to 4.2:1. Yarn samples were analyzed and the results are shown in Table 2. Tenacity improvement from about 0.26 N/tex (2.9 g/d) of Examples 6 and C2, to about 0.28 N/tex (3.2 grams/denier) was observed in both Examples 8 and C3. However, retained knot strength of C3 dropped to 27.7 % and coefficient of variation increased to 51.5 %. Surprisingly, the retained knot strength of Example 8 remained high at 58.9 % and variability improved to 6.8 %, despite the fact that tenacity was increased by raising the draw ratio relative to Example 6.

### Examples 9-10 and Comparative Example C4

A masterbatch of 30% Polymer G and 70% Polymer A was prepared as in Example 6. The masterbatch and a separate stream of Polymer A pellets were metered to a yarn extrusion line in proportions to produce yarns of 3.0, 1.5 and 0 % Polymer G. Samples of the 0.6 mm diameter yarns were tested and the results are shown in Table 3.

Table 3 data confirm that only low concentrations of PCTG in PCTA were needed to improve retained knot strength and did not adversely affect other properties. Although the unknotted tensile strength (7.7 kg (17 pounds)) of the yarn of Example 10 dropped relative to C4 (8.2 kg (18 pounds)), knot strength of the monofilament with only 1.5 % PCTG was much higher than of C4. The hydrolysis resistance of the yarns from blends remained excellent at greater than 95%. A comparable sample of PET yarn was not tested, however, its hydrolysis resistance is expected to be only about 80%.

Conversion factors into S.I.-units:
1 denier = ¹/₉ tex
1 gram per denier = 0.0885 N/tex
1 lb = 0.4536 kg

## Claims

1. A monofilament of a polymer blend consisting essentially of:
(a) 1 to 10 weight percent of a polyester selected from the group consisting of (1) polycarbonate and (2) glycol-modified copolyester comprising recurring units of copolymerized cyclohexane-1,4-dimethanol and copolymerized terephthalic acid, and recurring units of copolymerized glycol other than cyclohexane-1,4-dimethanol and copolymerized terephthalic acid; and
(b) a complementary amount to total 100 weight percent of acid-modified copolyester comprising recurring units of copolymerized cyclohexane-1,4-dimethanol and copolymerized terephthalic acid, and recurring units of copolymerized cyclohexane-1,4-dimethanol and copolymerized dicarboxylic acid other than terephthalic acid.

2. A monofilament according to claim 1, wherein said polyester is a glycol-modified copolyester comprising
50 to 95 mole % of recurring units of copolymerized cyclohexane-1,4-dimethanol and copolymerized terephthalic acid, and
a complementary amount to total 100 mole % of recurring units of a copolymerized bifunctional glycol having 2-20 carbon atoms, selected from the group consisting of linear, branched and cyclic aliphatic glycols and ether glycols; and copolymerized terephthalic acid; and
wherein said acid-modified copolyester comprises
50 to 95 mole % recurring units of copolymerized cyclohexane-1,4-dimethanol and copolymerized terephthalic acid, and
a complementary amount to total 100 mole % of recurring units of copolymerized cyclohexane-1,4-dimethanol and copolymerized isophthalic acid.

3. A monofilament according to claim 2, wherein said bifunctional glycol is ethylene glycol.

4. A monofilament according to claim 3, wherein the glycol-modified copolyester is present at 1 to 6 weight percent.

5. A monofilament according to claim 3, wherein the glycol-modified copolyester is present at 1.5 to 3 weight percent.

6. A monofilament according to claim 1, wherein said polyester is polycarbonate having recurring units of the following formula: wherein A is a divalent aromatic radical of bisphenol A; and
wherein said acid-modified copolyester comprises
50 to 95 mole % recurring units of copolymerized cyclohexane-1,4-dimethanol and copolymerized terephthalic acid, and
a complementary amount to total 100 mole % of recurring units of copolymerized cyclohexane-1,4-dimethanol and copolymerized isophthalic acid.

7. A monofilament according to claim 6, wherein the polycarbonate is present at 1 to 5 weight percent.

8. A papermaker's fabric comprising monofilaments of a polymer blend consisting essentially of:
(a) 1 to 10 weight percent of a polyester selected from the group consisting of (1) polycarbonate and (2) glycol-modified copolyester comprising recurring units of copolymerized cyclohexane-1,4-dimethanol and copolymerized terephthalic acid, and recurring units of copolymerized glycol other than cyclohexane-1,4-dimethanol and copolymerized terephthalic acid; and
(b) a complementary amount to total 100 weight percent of acid-modified copolyester comprising recurring units of copolymerized cyclohexane-1,4-dimethanol and copolymerized terephthalic acid, and recurring units of copolymerized cyclohexane-1,4-dimethanol and copolymerized dicarboxylic acid other than terephthalic acid.

9. A papermaker's fabric according to claim 8, wherein (a) is present from 1 to 6 weight percent and is a glycol-modified copolyester comprising
50 to 95 mole % of recurring units of copolymerized cyclohexane-1,4-dimethanol and copolymerized terephthalic acid, and
a complementary amount to total 100 mole % of recurring units of copolymerized ethylene glycol and copolymerized terephthalic acid; and
wherein said acid-modified copolyester comprises
50 to 95 mole % recurring units of copolymerized cyclohexane-1,4-dimethanol and copolymerized terephthalic acid, and
a complementary amount to total 100 mole % of recurring units of copolymerized cyclohexane-1,4-dimethanol and copolymerized isophthalic acid.

10. A papermaker's fabric according to claim 8, wherein (a) is present from 1 to 5 weight percent and is polycarbonate having recurring units of the following formula: wherein A is a divalent aromatic radical of bisphenol A; and
wherein said acid-modified copolyester comprises
50 to 95 mole % recurring units of copolymerized cyclohexane-1,4-dimethanol and copolymerized terephthalic acid, and
a complementary amount to total 100 mole % of recurring units of copolymerized cyclohexane-1,4-dimethanol and copolymerized isophthalic acid.

11. A method for making papermaker's fabric comprising forming said fabric from yarns including monofilament of a polymer blend consisting essentially of:
(a) 1 to 10 weight percent of a polyester selected from the group consisting of (1) polycarbonate and (2) glycol-modified copolyester comprising
recurring units of copolymerized cyclohexane-1,4-dimethanol and copolymerized terephthalic acid, and
recurring units of copolymerized glycol other than cyclohexane-1,4-dimethanol and copolymerized terephthalic acid; and
(b) a complementary amount to total 100 weight percent of acid-modified copolyester comprising
recurring units of copolymerized cyclohexane-1,4-dimethanol and copolymerized terephthalic acid, and
recurring units of copolymerized cyclohexane-1,4-dimethanol and copolymerized dicarboxylic acid other than terephthalic acid.

## Patentansprüche

1. Ein Monofilament einer Polymermischung, die im wesentlichen aus folgendem besteht:
(a) 1 bis 10 Gewichtsprozent eines Polyesters, das aus der Gruppe ausgewählt wurde, die aus (1) Polycarbonat und (2) glycolmodifiziertem Copolyester besteht, das periodische Einheiten von copolymerisiertem 1,4 Cyclohexan-Dimethanol und copolymerisierter Terephthalsäure, und periodische Einheiten von copolymerisiertem Glycol anders als 1,4 Cyclohexan-Dimethanol und copolymerisierter Terephthalsäure enthält; und
(b) einer ergänzenden Menge, um insgesamt 100 Gewichtsprozent auszumachen, von säuremodifiziertem Copolyester, das periodische Einheiten von copolymerisiertem 1,4 Cyclohexan-Dimethanol und copolymerisierter Terephthalsäure, und periodischen Einheiten von copolymerisiertem 1,4 Cyclohexan-Dimethanol und copolymerisierter Dicarbonsäure anders als Terephthalsäure aufweist.

2. Ein Monofilament nach Anspruch 1, worin genanntes Polyester ein glycolmodifiziertes Copolyester ist, das 50 bis 95 Mol % periodischer Einheiten von copolymerisiertem 1,4 Cyclohexan-Dimethanol und copolymerisierter Terephthalsäure, und
eine ergänzende Menge, um insgesamt 100 Mol % auszumachen, von periodischen Einheiten eines copolymerisierten bifuntionellen Glycols mit 2-20 Kohlenstoffatomen aufweist, das aus der Gruppe linearer, verzweigter und zyklisch aliphatischer Glycole und Ätherglycole ausgewählt wurde; und copolymerisierte Terephthalsäure umfaßt; und
worin genanntes säuremodifiziertes Copolyester 50 bis 95 Mol % periodischer Einheiten von copolymerisiertem 1,4 Cyclohexan-Dimethanol und copolymerisierter Terephthalsäure, und
eine ergänzende Menge, um insgesamt 100 Mol % auszumachen, periodischer Einheiten von copolymerisiertem 1,4 Cyclohexan-Dimethanol und copolymerisierter Isophthalsäure umfaßt.

3. Ein Monofilament nach Anspruch 2, worin genanntes bifunktionelles Glycol Ethylenglycol ist.

4. Ein Monofilament nach Anspruch 3, worin das glycolmodifizierte Copolyester mit 1 bis 6 Gewichtsprozent zugegen ist.

5. Ein Monofilament nach Anspruch 3, worin das glycolmodifizierte Copolyester mit 1,5 bis 3 Gewichtsprozent zugegen ist.

6. Ein Monofilament nach Anspruch 1, worin genanntes Polyester Polycarbonat ist, das periodische Einheiten der folgenden Formel aufweist: worin A ein zweiwertiges aromatisches Radikal von Bisphenol A ist; und
worin genanntes säuremodifiziertes Copolyester
50 bis 95 Mol % periodischer Einheiten von copolymerisiertem 1,4 Cyclohexan-Dimethanol und copolymerisierter Terephthalsäure, und
eine ergänzende Menge, um insgesamt 100 Mol % auszumachen, periodischer Einheiten von copolymerisiertem 1,4 Cyclohexan-Dimethanol und copolymerisierter Isophthalsäure umfaßt.

7. Ein Monofilament nach Anspruch 6, worin das Polycarbonat mit 1 bis 5 Gewichtsprozent zugegen ist.

8. Ein Papiermachergewebe, das Monofilamente einer Polymermischung umfaßt, die im wesentlichen aus folgendem besteht:
(a) 1 bis 10 Gewichtsprozent eines Polyesters, das aus der Gruppe ausgewählt wurde, die aus (1) Polycarbonat und (2) glycolmodifiziertem Copolyester besteht das periodische Einheiten von copolymerisiertem 1,4 Cyclohexan-Dimethanol und copolymerisierter Terephthalsäure, und periodische Einheiten von copolymerisiertem Glycol anders als 1,4 Cyclohexan-Dimethanol und copolymerisierter Terephthalsäure enthält; und
(b) einer ergänzenden Menge, um insgesamt 100 Gewichtsprozent auszumachen, von säuremodifiziertem Copolyester, das periodische Einheiten von copolymerisiertem 1,4 Cyclohexan-Dimethanol und copolymerisierter Terephthalsäure, und periodischen Einheiten von copolymerisiertem 1,4 Cyclohexan-Dimethanol und copolymerisierter Dicarbonsäure anders als Terephthalsäure aufweist.

9. Ein Papiermachergewebe nach Anspruch 8, worin (a) von 1 bis 10 Gewichtsprozent zugegen ist und ein glycolmodifiziertes Copolyester ist, das
50 bis 95 Mol % periodischer Einheiten von copolymerisiertem 1,4 Cyclohexan-Dimethanol und copolymerisierte Terephthalsäure, und
eine ergänzende Menge, um insgesamt 100 Mol % auszumachen, periodischer Einheiten von copolymerisiertem Ethylenglycol und copolymerisierter Terephthalsäure umfaßt; und
worin genanntes säuremodifiziertes Copolyester
50 bis 95 Mol % periodischer Einheiten von copolymerisiertem 1,4 Cyclohexan-Dimethanol und copolymerisierte Terephthalsäure, und
eine ergänzende Menge, um insgesamt 100 Mol % auszumachen, periodischer Einheiten von copolymerisiertem 1,4 Cyclohexan-Dimethanol und copolymerisierter Isophthalsäure umfaßt.

10. Ein Papiermachergewebe nach Anspruch 8, worin (a) von 1 bis 5 Gewichtsprozent zugegen ist und Polycarbonat ist, das periodische Einheiten der folgenden Formel aufweist: worin A ein zweiwertiges aromatisches Radikal von Bisphenol A ist; und
worin genanntes säuremodifiziertes Copolyester
50 bis 95 Mol % periodischer Einheiten von copolymerisiertem 1,4 Cyclohexan-Dimethanol und copolymerisierter Terephthalsäure, und
eine ergänzende Menge, um insgesamt 100 Mol % auszumachen, periodischer Einheiten von copolymerisiertem 1,4 Cyclohexan-Dimethanol und copolymerisierter Isophthalsäure umfaßt.

11. Ein Verfahren für das Herstellen eines Papiermachergewebes, welches das Formen des genannten Gewebes aus Garnen umfaßt, die Monofilament einer Polymermischung einschließen, die im wesentlichen aus folgendem besteht:
(a) 1 bis 10 Gewichtsprozent eines Polyesters, das aus der Gruppe ausgewählt wurde, die aus (1) Polycarbonat und (2) glycolmodifiziertem Copolyester besteht, das
periodische Einheiten von copolymerisiertem 1,4 Cyclohexan-Dimethanol und copolymerisierter Terephthalsäure, und
periodische Einheiten von copolymerisiertem Glycol anders als 1,4 Cyclohexan-Dimethanol und copolymerisierter Terephthalsäure enthält; und
(b) einer ergänzenden Menge, um insgesamt 100 Gewichtsprozent auszumachen, von säuremodifiziertem Copolyester,
das periodische Einheiten von copolymerisiertem 1,4 Cyclohexan-Dimethanol und copolymerisierter Terephthalsäure, und
periodischen Einheiten von copolymerisiertem 1,4 Cyclohexan-Dimethanol und copolymerisierter Dicarbonsäure anders als Terephthalsäure aufweist.

## Revendications

1. Un monofilament composé d'un mélange de polymères, composé essentiellement :
(a) pour 1% à 10% (de sa masse), d'un polyester choisi dans le groupe composé de (1) un polycarbonate et (2) un copolyester modifié au glycol comprenant des unités récurrentes de cyclohéxane-1,4-diméthanol copolymérisé et d'acide théréphtalique copolymérisé, et des unités récurrentes d'un glycol copolymérisé autre que le cyclohéxane-1, 4-diméthanol et d'acide théréphtalique copolymérisé; et
(b) d'un pourcentage complémentaire (afin d'arriver à un total de 100% de la masse du monofilament) de copolyester modifié à l'acide comprenant des unités récurrentes de cyclohéxane-1, 4-diméthanol copolymérisé et d'acide théréphtalique copolymérisé, et des unités récurrentes de cyclohéxane-1, 4-diméthanol copolymérisé et d'un acide dicarboxylique copolymérisé autre que l'acide théréphtalique.

2. Un monofilament ainsi revendiqué à la revendication 1, dans lequel ledit polyester est un copolyester modifié au glycol composé :
pour 50 à 95% du total molaire, d'unités récurrentes de cyclohéxane-1, 4-diméthanol copolymérisé et d'acide théréphtalique copolymérisé, et
d'un pourcentage complémentaire (afin d'arriver à un total de 100% du total molaire) d'unités récurrentes d'un glycol copolymérisé bifonctionnel comportant de 2 à 20 atomes de carbone, et choisi dans le groupe comprenant les glycols aliphatiques linéaires, ramifiés et cycliques et les glycols ethylènes; et de l'acide théréphtalique copolymérisé; et
dans lequel ledit copolyester modifié à l'acide comprend
de 50 à 95% du total molaire, d'unités récurrentes de cyclohéxane-1, 4-diméthanol copolymérisé et d'acide théréphtalique copolymérisé, et
un pourcentage complémentaire (afin d'arriver à un total de 100% du total molaire) d'unités récurrentes de cyclohéxane-1, 4-diméthanol copolymérisé et d'acide isophtalique copolymérisé.

3. Un monofilament ainsi revendiqué à la revendication 2, dans lequel ledit glycol bifonctionnel est de l'éthylène glycol.

4. Un monofilament ainsi revendiqué à la revendication 3, dans lequel le copolyester modifié au glycol est présent à hauteur de 1 à 6% de la masse totale.

5. Un monofilament ainsi revendiqué à la revendication 3, dans lequel le copolyester modifié au glycol est présent à hauteur de 1,5 à 3% de la masse totale.

6. Un monofilament ainsi revendiqué à la revendication 1, dans lequel ledit polyester est un polycarbonate comprenant des unités récurrentes dont la formule est la suivante: où A est un radical aromatique divalent du bisphénol A; et
dans lequel ledit copolyester modifié à l'acide comprend
de 50 à 95%, en moles, d'unités récurrentes de cyclohéxane-1, 4-diméthanol copolymérisé et d'acide théréphtalique copolymérisé, et
un pourcentage complémentaire (afin d'arriver à un total de 100% du total molaire) d'unités récurrentes de cyclohéxane-1, 4-diméthanol copolymérisé et d'acide isophtalique copolymérisé.

7. Un monofilament ainsi revendiqué à la revendication 6, dans lequel le polycarbonate est présent à hauteur de 1 à 5% de la masse.

8. Un tissu destiné à la fabrication du papier comprenant des monofilaments composés d'un mélange de polymères dont la composition est essentiellement la suivante:
(a) un pourcentage inclus entre 1 et 10% de la masse du mélange est un polyester issu du groupe composé de (1) un polycarbonate et (2) un copolyester modifié au glycol comprenant des unités récurrentes de cyclohéxane-1, 4-diméthanol copolymérisé et d'acide théréphtalique copolymérisé, et des unités récurrentes d'un glycol copolymérisé autre que le cyclohéxane-1, 4-diméthanol et d'acide théréphtalique copolymérisé; et
(b) un pourcentage complémentaire (afin d'arriver à un total de 100% de la masse) d'un copolyester modifié à l'acide comprenant des unités récurrentes de cyclohéxane-1, 4-diméthanol copolymérisé et d'acide théréphtalique copolymérisé, et des unités récurrentes de cyclohéxane-1, 4-diméthanol copolymérisé et d'un acide dicarboxylique copolymérisé autre que l'acide théréphtalique.

9. Un tissu destiné à la fabrication du papier ainsi revendiqué à la revendication 8, dans lequel l'élément (a) représente de 1 à 6% de la masse et est un copolyster modifié au glycol comprenant
de 50 à 95% du total molaire d'unités récurrentes de cyclohéxane-1, 4-diméthanol copolymérisé et d'acide théréphtalique copolymérisé, et
un pourcentage complémentaire (afin d'arriver à un total de 100% du total molaire) d'unités récurrentes d'éthylène glycol copolymérisé et d'acide théréphtalique copolymérisé; et
dans lequel ledit copolyester modifié à l'acide comprend
de 50 à 95% du total molaire d'unités récurrentes de cyclohéxane-1, 4-diméthanol copolymérisé et d'acide théréphtalique copolymérisé, et
un pourcentage complémentaire (afin d'arriver à un total de 100% du total molaire) d'unités récurrentes de cyclohéxane-1, 4-diméthanol copolymérisé et d'acide isophtalique copolymérisé.

10. Un tissu destiné à la fabrication du papier ainsi revendiqué à la revendication 8, dans lequel (a) est présent à hauteur de 1 à 5% de la masse et est un polycarbonate comprenant des unités récurrentes dont la formule est la suivante: où A est un radical aromatique divalent du bisphénol A; et
dans lequel ledit copolyester modifié à l'acide comprend
de 50 à 95%, en moles, d'unités récurrentes de cyclohéxane-1, 4-diméthanol copolymérisé et d'acide théréphtalique copolymérisé, et
un pourcentage complémentaire (afin d'arriver à un total de 100% du total molaire) d'unités récurrentes de cyclohéxane-1, 4-diméthanol copolymérisé et d'acide isophtalique copolymérisé

11. Une méthode visant à produire un tissu destiné à la fabrication du papier, consistant en particulier à assembler ledit tissu à partir de fils comprenant un monofilament composé d'un mélange de polymères composé essentiellement:
(a) pour 1% à 10% (de sa masse) d'un polyester choisi dans le groupe composé de (1) un polycarbonate et (2) un copolyester modifié au glycol comprenant
des unités récurrentes de cyclohéxane-1,4-diméthanol copolymérisé et d'acide théréphtalique copolymérisé, et
des unités récurrentes d'un glycol copolymérisé autre que le cyclohéxane-1, 4-diméthanol et d'acide théréphtalique copolymérisé; et
(b) d'un pourcentage complémentaire (afin d'arriver à un total de 100% de la masse du monofilament) de copolyester modifié à l'acide comprenant
des unités récurrentes de cyclohéxane-1, 4-diméthanol copolymérisé et d'acide théréphtalique copolymérisé, et
des unités récurrentes de cyclohéxane-1, 4-diméthanol copolymérisé et d'un acide dicarboxylique copolymérisé autre que l'acide théréphtalique.
